

March 13, 1945.

F. R. HENSEL ET AL

2,371,240

ELECTRIC CONTACT

Filed May 27, 1943

*Fig. 1*



*Fig. 2*



Franz R. Hensel  
Kenneth L. Emmert  
James W. Wiggs  
INVENTORS

BY *Robbin + Carlson*

ATTORNEYS

## UNITED STATES PATENT OFFICE

2,371,240

## ELECTRIC CONTACT

Franz R. Hensel, Kenneth L. Emmert, and James W. Wiggs, Indianapolis, Ind., assignors to P. R. Mallory & Co., Inc., Indianapolis, Ind., a corporation of Delaware

Application May 27, 1943, Serial No. 488,746

4 Claims. (Cl. 200—166)

This invention relates to electric contacts.

An object of the invention is to improve electric contacts and the composition thereof.

Other objects of the invention will be apparent from the description and claims.

In the drawing Figure 1 illustrates a contact combination formed of contacts of the present invention and Figure 2 shows a contact combination in which one of the contacts is of the composition of the present invention and the co-operating contact is formed of another material.

The present invention contemplates an electric contact formed of an alloy containing gold, silver, and one or both of the metals cadmium and zinc.

The ingredients may be present in the following ranges of proportions, by weight:

|                                    | Per cent  |
|------------------------------------|-----------|
| Cadmium, zinc or cadmium plus zinc | 0.5 to 20 |
| Silver                             | 1 to 50   |
| Gold                               | 40 to 98  |

Small proportions of other ingredients, such as copper, platinum, palladium, nickel, cobalt, indium, tin, may in some cases be present. These materials, if present, may be substituted for an equal proportion of silver in proportions of 0.1 to 20% of the alloy.

Alloys of gold, silver and cadmium form the preferred contact material.

The preferred composition range is

|         | Per cent |
|---------|----------|
| Cadmium | 1 to 15  |
| Silver  | 3 to 30  |
| Gold    | Balance  |

The following specific contact materials have been found to be very satisfactory.

(1) Per cent

|         |         |
|---------|---------|
| Cadmium | 3       |
| Silver  | 25      |
| Gold    | Balance |

(2) Per cent

|         |         |
|---------|---------|
| Cadmium | 5       |
| Zinc    | 3       |
| Silver  | 10      |
| Gold    | Balance |

(3) Per cent

|         |         |
|---------|---------|
| Cadmium | 10      |
| Silver  | 20      |
| Gold    | Balance |

The contact alloys are readily produced by conventional alloying methods, including standard melting procedures, manufacture by powder metallurgy, plating and subsequent diffusion etc. The compositions most suitable for electrical contact purposes fall within the ternary solid solu-

tion range of gold-silver-cadmium. It has been found advantageous to have a homogeneous matrix since this will assist greatly in decreasing the tendency to either welding of contacts or material transfer.

The present contact materials made of gold base alloys have the disadvantage of high material transfer usually in the form of needles. Such needles will result in ultimate failure of 10 the contacts since the needles will cause a mechanical interlocking into the crater of the mating contact. The improved alloys of the present invention eliminate these difficulties and thereby provide contacts which can be operated for long 15 periods of time. The noble characteristics of the alloys permit operation at extremely low contact pressures without creating films on the contact surfaces resulting in high contact resistance. The alloys are also applicable to control equipment which has to operate in industrial atmospheres usually contaminated with sulfur since they will resist tarnishing or corroding.

In certain D. C. applications it has been found advantageous to operate the contacts of the present invention against a differential contact material such as a silver base, platinum and/or palladium base or a refractory base composition. The refractory base metals may be either swaged tungsten compositions or Elkonites which are compound metals having a refractory base and containing lower melting point materials such as copper, silver and gold.

Figure 1 of the drawing shows a pair of co-operating contacts 1 and 3 both formed of the alloy of the present invention brazed or welded to support arms 2 and 4 respectively. Figure 2 shows contact 5 formed of the composition of the present invention mounted on support arm 6 for cooperation with another contact 7 formed of another composition mounted on support arm 8.

While specific embodiments of the invention have been described, it is intended to cover the invention broadly within the spirit and scope of the appended claims.

What is claimed is:

1. An electric contact formed of an alloy of 0.5 to 20% of an element selected from the group consisting of cadmium and zinc, 1 to 50% silver and 40 to 98% gold.

2. An electric contact formed of an alloy of 1 to 15% cadmium, 3 to 30% silver and the balance gold.

3. An electric contact formed of an alloy of 3% cadmium, 25% silver and the balance gold.

4. An electric contact formed of an alloy of 10% cadmium, 20% silver and the balance gold.

FRANZ R. HENSEL.

KENNETH L. EMMERT.

JAMES W. WIGGS.